

## UNITED STATES PATENT OFFICE

HERBERT A. LUBS, OF PENNS GROVE, NEW JERSEY, AND ARTHUR L. FOX, OF WILMINGTON, DELAWARE, ASSIGNEES TO E. I. DU PONT DE NEMOURS & COMPANY, OF WILMINGTON, DELAWARE, A CORPORATION OF DELAWARE

## PROCESS OF CONCENTRATING ORES BY FLOTATION

No Drawing.

Application filed December 13, 1927. Serial No. 239,816.

- This invention relates to improvements in the process of concentrating ores and minerals by flotation, particularly by the use of certain types of compounds which have not hitherto been employed for this purpose. It has been found that the concentration of ores by flotation can be greatly facilitated if we use in the flotation operation certain organic compounds containing the group—SH.
- 10 It has been discovered that marked flotation effects are obtained with organic compounds containing the group—SH, in which H may be replaced by a metal, as the alkali metals or lead, said group being attached to
- 15 a carbon of an organic radical which, if it is an aryl radical, is preferably free from amino groups ortho to the mercapto group, said carbon being in turn attached to at least one other carbon atom or to hydrogen.
- 20 All of these compounds are effective but some to a less degree than others. Many of them are extremely powerful flotation agents. The aliphatic mercaptans, for example, are excellent flotation agents, whether they are
- 25 normal or branch-chain compounds. The cyclic compounds are also effective, such for example as cyclo propyl, cyclo hexyl mercaptans, etc. The number of aromatic mercaptans which can be satisfactorily employed
- 30 is also very large. The phenyl mercaptans and their derivatives, such for example as the halogenated, alkyl, nitro, hydroxy, carboxy, sulfonic acid, etc., derivatives may be used, or the naphthyl mercaptans and their
- 35 derivatives may be employed, or such compounds as aryl phenyl or aryl naphthyl derivatives, also the mercaptans in the anthracene and anthraquinone series are effective flotation agents, such for example as anthraquinone - alpha - mercaptan. Partially or completely hydrogenated cyclic compounds are also useful. As examples we may mention decahydro-naphthyl-mercaptop, tetrahydro-naphthyl - mercaptan. Heterocyclic
- 45 compounds are also effective, such for ex-

ample as thiophene mercaptan, furyl mercaptan, pyridyl mercaptan, thionthrene mercaptan, quinoline mercaptan. Such compounds also as benzyl mercaptan and furfuryl mercaptan may also be used.

In order to illustrate the effectiveness of these compounds, the following examples of processes involving their employment in representative flotation operations are submitted:

## Example I

Five hundred grams of copper ore (0.95% Cu) from the Inspiration Consolidated Copper Company were ground in a pebble mill with 450 cc. of water and 0.35 g. of hydrated lime. This pulp was transferred to a mechanically agitated flotation machine and conditioned therein for 1 minute with pine oil and .005 g. of ethyl mercaptan. Water was then added to give a pulp of approximately 20% solids. This dilution caused circulation of the pulp thru the spitz, and froth formation. The froth was removed for 10 minutes. A similar test was made using isooamyl mercaptan. The results are tabulated below:

| Product           | Amt.,<br>lbs./ton | Percent<br>Cu in<br>concent-<br>rate | Percent<br>Cu in<br>tailings | Percent<br>Cu re-<br>covered |
|-------------------|-------------------|--------------------------------------|------------------------------|------------------------------|
| Ethyl mercaptan   | .025              | 13.23                                | 0.33                         | 69.3                         |
| Isoamyl mercaptan | .050              | 11.55                                | 0.36                         | 67.2                         |

## Example II

Five hundred grams of copper ore (0.95% Cu) from the Inspiration Consolidated Copper Company were ground in the pebble mill with 450 cc. of water and 0.35 g. of hydrated lime. This pulp was divided into three parts and transferred to mechanically agitated flotation machines and each part conditioned therein for one minute with pine oil and one of the aromatic mercaptans listed in the following tabulation. Water was

then added to give a pulp of approximately 20% solids. This dilution caused circulation of the froth thru the spitz, and froth formation. The froth was removed for 10 minutes. The results are indicated below:

|    | Product                         | Amt., lbs./ton | Per cent Cu in concentrate | Per cent Cu in tailings | Per cent Cu recovered |
|----|---------------------------------|----------------|----------------------------|-------------------------|-----------------------|
| 10 | Blank test—pine oil alone       | 0.16           | 2.28                       | 0.90                    | 7.0                   |
|    | p-thiocresol (with pine oil)    | 0.014          | 22.00                      | 0.39                    | 59.7                  |
|    | Thiophenol (with pine oil)      | 0.006*         | 10.70                      | 0.32                    | 68.0                  |
|    | Thio-b-naphthol (with pine oil) | 0.008*         | 9.80                       | 0.45                    | 54.5                  |

\*0.24 lb. of pine oil used, in other tests 0.16 lb. used.

15 The higher amount of pine oil used caused the inclusion of more gangue in the concentrate thereby lowering the percent Cu therein.

20 When the process is carried out with the above reagents, the amount used can be even less than the figures given. Thiocresol, for example, even in an amount as low as 0.001 lb. per ton of ore, shows strong flotation action.

25 In addition to the compounds discussed in the above examples, we have tested and found satisfactory many other such compounds, for example,

30 iso-amyl mercaptan.

methyl-mercaptan.

propyl-mercaptan.

n-butyl-mercaptan.

35 isopropyl-mercaptan.

p-dichlor-phenyl-mercaptan.

p-dichlor-phenyl-dimercaptan.

o-dichlor-phenyl-dimercaptan.

p-methyl-iso-propyl-phenyl-mercaptan.

mercapto-ortho-cresol.

40 benzyl-mercaptan.

Of the many compounds which fall within the scope of our invention, thiophenol may be mentioned as one of our preferred embodiments.

45 We have also found that remarkably strong flotation action is obtained with compounds of the general type



in which H may be replaced by a metal, and in which R is an organic radical, to a carbon of which is attached the group



60 The carrying into effect of the process with several such reagents is illustrated below.

### Example III

65 Five hundred grams of copper ore (0.95% Cu) from the Inspiration Copper Company were ground in a pebble mill with 450 cc.

water and 0.35 g. hydrated lime. The pulp was then transferred to a mechanically agitated flotation machine, and conditioned for one minute with pine oil and one of the flotation agents indicated below. Water was then added to give a pulp of approximately 20% solids. This caused circulation of the pulp through the spitz, with froth formation. The froth was removed for 10 minutes.

70 The amounts of reagent used and the recovery of copper are shown below in connection with each specific reagent employed:

|                                                   | Amt. reagent, lbs. per ton | Per cent Cu in conc. | Per cent Cu in tailings | Per cent Cu recovered |
|---------------------------------------------------|----------------------------|----------------------|-------------------------|-----------------------|
| Mg salt of dithiobenzoic acid (with pine oil)     | 0.02                       | 11.1                 | 0.34                    | 69.1                  |
| Crude dithiobenzoic acid (with pine oil)          | 0.08                       | 17.0                 | 0.30                    | 60.0                  |
| Zinc salt of dithiobenzoic acid (with pine oil)   | 0.04                       | 12.7                 | 0.36                    | 63.6                  |
| Sodium salt of dithiobenzoic acid (with pine oil) | 0.02*                      | 5.8                  | 0.48                    | 53.4                  |
| Na salt of dithiopropionic acid (with pine oil)   | 0.05                       | 14.9                 | 0.55                    | 41.9                  |
| Blank test (pine oil alone)                       | 0.16                       | 2.3                  | 0.90                    | 7.0                   |

\*0.24 lb. of pine oil used instead of usual 0.16 lb., the use of more pine oil causing the inclusion of more gangue in the concentrate, thereby lowering the percent copper therein.

Many other compounds of the type



may also be used. As examples we may mention dithiosalicylic acid, dithiotoluic acid, p-methoxy-dithiobenzoic acid, dithiobutyric acid, dithiogluconic acid, dithioacetic acid, dithiovaleric acid, or their salts. Naturally compounds of this type are not all equally effective. Among our preferred compounds of this particular group are the magnesium and sodium salts of dithiobenzoic acid and the sodium salt of dithiobenzoic acid.

100 The new flotation agents are also, in general, adapted for use in selective flotation operations but some of them, for example, thiophenol and thiocresol, and the magnesium salt of dithiobenzoic acid, have the property, to a very remarkable degree, of selective flotation and may be employed to advantage, for example, in floating copper sulfide in preference to iron sulfide.

110 It is obvious from the foregoing illustrations that the class of compounds described constitutes unusually effective flotation agents. These compounds are adapted for use over a wide range of conditions. Where employed for selective flotation with complex ores the ores may of course contain more than two minerals and the process of selection carried out by merely repeating the flotation step for each ore it is desired to recover.

120 The usual conditioning agents may, of course, be employed with the new flotation agents, as illustrated in the examples.

It will be understood that the invention is not limited to the specific classes of compounds or the specific compounds themselves mentioned above for illustrative purposes, but many other compounds not mentioned above, but which come within the scope of the following claims, may be employed. It is to be understood that where the terms aliphatic, aromatic and heterocyclic are employed in the claims they may indicate either substituted or unsubstituted groups.

We claim:

1. In the concentration of ores and minerals by flotation, the step which comprises subjecting the ore, in the form of a pulp, to a froth flotation operation in the presence of a compound of the type



20 in which H may be replaced by a metal, and R is an organic radical, to a carbon of which the group



is attached.

2. In the concentration of ores and minerals by flotation, the step which comprises subjecting the ore, in the form of a pulp, to a froth flotation operation in the presence of a compound of the type



35 in which H may be replaced by a metal, and R is an aromatic radical, to a carbon of which the group



is attached.

3. In the concentration of ores and minerals by flotation, the step which comprises subjecting the ore, in the form of a pulp, to a froth flotation operation in the presence of a compound of the type



50 in which H may be replaced by a metal, and R is a radical of the group consisting of aliphatic, aromatic and heterocyclic radicals, to a carbon of which the group



55 is attached.

4. In the concentration of ores and minerals by froth flotation, the step which comprises subjecting the ore, in the form of a pulp, to a flotation operation in the presence of a dithiofuroic acid compound.

5. In the concentration of ores and minerals by froth flotation, the step which comprises subjecting the ore, in the form of a pulp, to a flotation operation in the presence of a salt of dithiofuroic acid.

6. In the concentration of ores and minerals by froth flotation, the step which comprises subjecting the ore, in the form of a pulp, to a flotation operation in the presence of a compound of the group consisting of dithiofuroic acid and dithiobenzoic acid compounds.

7. In the process of concentrating ores and minerals, the step which comprises subjecting an ore containing copper and iron, said ore being in the form of a pulp, to a froth flotation operation in the presence of an organic compound adapted to raise copper sulfide and depress iron sulfide, said compound being of the type



85 in which H may be replaced by a metal, and R is an organic radical, to a carbon of which the group



is attached.

8. In the process of concentrating ores and minerals, the step which comprises subjecting an ore, containing at least two metals, in the form of a pulp to a froth flotation operation in the presence of a compound adapted to raise one metal and depress another, said compound being of the group consisting of dithiofuroic acid and dithiobenzoic acid.

90 In testimony whereof we affix our signatures.

HERBERT A. LUBS.  
ARTHUR L. FOX.

95

100

105

110

115

120

125

130